

## UNITED STATES PATENT OFFICE

2,223,128

## LUBRICATING COMPOSITION

Carl F. Prutton, East Cleveland, Ohio, assignor, by  
mesne assignments, to The Lubri-Zol Develop-  
ment Corporation, Cleveland, Ohio, a corpora-  
tion of Delaware

No Drawing. Application May 1, 1940,  
Serial No. 332,781

5 Claims. (Cl. 252—37)

This invention relates, as indicated, to lubricating compositions and more particularly to lubricating compositions which are predominantly hydrocarbon oil, the properties of which affecting its use for particular purposes are improved by the addition of materials which are particularly effective in rendering the lubricants suitable for use under conditions of extreme stress as imposed by high temperatures, high loads, etc.

10 In my co-pending applications, Ser. Nos. 737,070, filed July 26, 1934; 216,153, filed June 27, 1938; and 245,226, filed December 12, 1938, I have disclosed a broad class of lubricating compositions of general utility, particularly in the field 15 of use where extreme service conditions are encountered.

My present invention relates to the discovery that a certain class of such materials is particularly suitable for use in lubricants subjected to 20 conditions of extreme stress such as those involved in the lubrication of heavily loaded gears, and in the lubrication of internal combustion engines operating under severe service conditions; for example, those encountered by internal 25 combustion engines particularly of the aviation and Diesel types.

It is the principal object of my invention, therefore, to provide a lubricating composition which is especially suited for the purposes described.

Other objects of my invention will appear as the description proceeds.

To the accomplishment of the foregoing and related ends, said invention, then, consists of 35 the means hereinafter fully described and particularly pointed out in the claims; the following description setting forth in detail certain approved combinations of ingredients embodying my invention, such disclosed means constituting, however, but one of various forms in which the principle of the invention may be used.

Broadly stated, this invention comprises the provision of a lubricating composition for the 45 purposes specified, characterized by the fact that the same contains a lubricating oil, preferably of the hydrocarbon type, as a major constituent with the properties of such composition affecting its use as a lubricant, especially under the 50 conditions specified, by the incorporation there-

in of a minor amount, based on the amount of lubricating oil present, of a stable, oil-soluble salt of an aromatic acid of the type which may be produced by condensing chlorbenzene with oleic acid.

## THE OIL BASE

The oil base of my lubricating compositions is a lubricating oil of the type best suited for the particular use for which the ultimate composition is designed. When the lubricating compositions of my invention are designed for the lubrication of automobiles, the oil base will of course preferably consist of a refined mineral lubricating oil of lubricating viscosity for the particular point of application. In other words, a conventional gear oil may be used for the lubrication of the gears and generally a lighter, more highly refined, oil will be used in the crank case.

This invention is applicable to lubricating compositions in which the base may consist 20 either entirely or in part of synthetic oils, hydrogenated oils, and volatilized oils.

The oil base may also desirably contain other well known constituents such as those which improve the oiliness, pour point, cold test, and 25 oxidation properties, etc., of the oil. In general, compositions of our invention may be employed with any commercially available addition agents for the above defined purposes since they are generally compatible with the same in the 30 amounts usually used.

## THE ADDITION AGENTS

As previously indicated, the addition agents of the lubricating compositions of my present invention may be broadly defined as stable oil soluble salts of aromatic acids of the type which may be produced by condensing chlorbenzene with oleic acid. Such salts may be either organic 35 or inorganic, the metallic salts being usually preferred.

The preferred metallic salts for use in such composition may be more specifically defined as those metallic salts of an aromatic acid of the 45 type which may be produced by condensing chlorbenzene with oleic acid, which metallic salts are of the type in which the metal is present in divalent form.

Among the divalent metal salts thus included 50

in the preferred class of addition agents are calcium chlorphenyl stearate, cobalt chlorphenyl stearate, nickel chlorphenyl stearate, magnesium chlorphenyl stearate, stannous chlorphenyl stearate, cupric chlorphenyl stearate and cadmium chlorphenyl stearate.

Below will be found, set out in detail, the method of preparation of certain examples of my invention with results secured by the use of the same in actual engine lubrication at carefully controlled conditions in order to show comparative results.

The salts used in the examples below were all prepared from chlorphenyl stearic acid which was made as follows:

357 parts of monochlor benzene were placed in a flask equipped with an agitating device, and 46.5 parts of aluminum chloride added. Then 100 parts of oleic acid were run in very slowly so as to maintain the temperature below 35° C. The temperature was then maintained at about 35° C. for an additional period of one hour. The contents of the flask were then added to a mixture of crushed ice and hydrochloric acid to destroy the complex. The product was washed with hot water and subjected to a distillation under a vacuum of 3 millimeters of mercury absolute pressure. The distillate coming over at a temperature below 120° C. (thermometer bulb in vapor, pressure 3 mm. Hg.) was discarded. The distillate coming over at temperatures between 120 and 275° C. was collected as the final product. The bulk of the distillate came over within a temperature range of 200 to 210° C.

35 The oleic acid used had the following characteristics:

|                                                   |            |
|---------------------------------------------------|------------|
| Iodine No. (Wijs') .....                          | 85         |
| Acid number .....                                 | 194        |
| 40 The product had the following characteristics: |            |
| Iodine No. (Wijs') .....                          | 4-8        |
| Acid number .....                                 | 155-165    |
| Percent chlorine .....                            | 6.0 to 5.5 |

#### 45 EXAMPLES

##### Example I

A blend of 1.33% calcium chlorphenyl stearate in a mineral lubricating oil of naphthenic type was prepared by dissolving 1.29% of chlorphenyl stearic acid in the oil, adding a 10% excess of calcium hydroxide and heating with agitation to 325° F. for 1½ hours. The blend was then 55 filtered after adding 2% of clay as a filter aid.

##### Example II

A blend of 1% of calcium chlorphenyl stearate in the same mineral lubricating oil as used 60 in Example I was prepared as follows:

300 parts by volume of chlorphenyl stearic acid were dissolved in 3000 parts of a 1% solution of sodium hydroxide. This mixture was heated to 85° C. for about 45 minutes and to the solution of sodium chlorphenyl stearate thus obtained 700 parts of a mineral lubricating oil were added. This oil was a Mid-Continent pale oil having a viscosity of approximately 300 SUS at 100° F. The oil and sodium chlorphenyl stearate 70 solution were agitated together at 85° C. for about 15 minutes. 300 parts of a 15.85% solution of calcium chloride was then added and the mixture stirred for 15 minutes with the temperature maintained at 85° C. The mixture was then 75 allowed to stand until it had separated into two

layers. The aqueous layer was discarded and the oil layer was then washed twice with 3000 parts of hot water and the moisture removed by heating to a temperature of 125° C. for two hours.

This procedure produced a concentrate containing approximately 30% of calcium chlorphenyl stearate in mineral oil. 3½% of this concentrate was incorporated in the mineral lubricating oil to produce the final blend.

##### Example III

A blend of 1% of magnesium chlorphenyl stearate in the same mineral lubricating oil as used in Example I was prepared by the same method as described in Example II except that an equivalent amount of magnesium chloride was used instead of calcium chloride.

##### Example IV

A blend of 1% of nickel chlorphenyl stearate in the same mineral lubricating oil as used in Example I was prepared by the same method as used in Example II, except that an equivalent amount of nickel nitrate was used instead of calcium chloride.

##### Example V

A blend of 1% of cobalt chlorphenyl stearate in the same lubricating oil as used in Example I was prepared by the same method as used in Example II except that an equivalent amount of cobaltous chloride was used instead of calcium chloride.

##### Example VI

A blend of .25% of cobalt chlorphenyl stearate in a highly solvent-extracted Mid-Continent motor oil was prepared by dissolving in the mineral oil .833% of the same concentrate used in Example V.

#### ENGINE TESTS

Tests were made of the mineral lubricating oils used in the above examples and of the blends, by means of a 2½ H. P. single-cylinder, liquid-cooled, four cycle gasoline engine, rated at 1800 R. P. M. The procedure used was as follows:

The engine was loaded by means of a fan-type brake which applied a load of 1½ H. P. at 1600 R. P. M. The engine was run for ten minutes at 1200 R. P. M. and then the speed was increased to 1600 R. P. M. The following conditions were maintained constant during the remainder of the test:

|                           |          |     |
|---------------------------|----------|-----|
| Coolant temperature ..... | °F ..... | 345 |
| Oil temperature .....     | °F ..... | 225 |
| Air fuel ratio .....      | 12.7:1   | 60  |

The engine was stopped at 30 hour periods for inspection of piston, piston skirt, piston rings, connecting rod bearings, etc. The engine was equipped with removable connecting-rod bearings consisting of lead-bronze with a steel backing. These bearings were weighed at the beginning of the test and at each 30 hour inspection period. Before each new test, the engine was thoroughly cleaned and equipped with new piston, piston rings and with new connecting rod bearings.

The characteristics of the mineral oils used to make the blends of Examples I to VI, and the characteristics of the blends are shown in 75

the table below. The results of the engine test described above are also shown in the table.

containing rather high percentages of the addition agents. Such concentrates may be employed

| 5  | Example number                        |            | I          | II        | III       | IV        | V         |               | VI         | 5            |
|----|---------------------------------------|------------|------------|-----------|-----------|-----------|-----------|---------------|------------|--------------|
| 10 | Type of oil                           | Naphthenic | Naphth.    | Naphth.   | Naphth.   | Naphth.   | Naphth.   | Solv. Ext.    | Solv. Ext. | 10           |
| 15 | Addition agent                        | None       | CaCPS 1.33 | CaCPS 1.0 | MgCPS 1.0 | NiCPS 1.0 | CoCPS 1.0 | None          | CoCPS 0.25 | 15           |
| 10 | Percent ash                           | 0          | .14        | 0.07      | 0.06      | 0.12      | 0.12      | 0             | 0.03       |              |
|    | Acid number                           | 0.05       | .34        | 0.31      | 1.24      | 0.34      | 1.35      | 0.04          | 0.28       |              |
|    | Conradson carbon, percent             | .09        | .37        | 0.33      | 0.22      | 0.33      | 0.31      | 0.24          | 0.35       |              |
|    | Viscosity at 210° F                   | 55.3       | 59.2       | 56.0      | 57.7      | 59.2      | 72.2      | 67.5          | 86.0       |              |
|    | Viscosity at 100° F                   | 601        |            |           |           |           |           | 622           |            |              |
|    | A. P. I. Gravity                      | 19.7       |            |           |           |           |           | 28.4          |            |              |
|    | Flash Point, ° F                      | 320        |            |           |           |           |           |               |            |              |
|    | Fire point, ° F                       | 430        |            |           |           |           |           |               |            |              |
| 15 | Pour point, ° F                       | -5         |            |           |           |           |           |               |            |              |
|    | N. P. A. Color                        | 2          |            |           |           |           |           |               |            |              |
|    | <i>Engine test</i>                    |            |            |           |           |           |           |               |            |              |
|    | Piston condition at—                  |            | D          | B<br>C    | B<br>C    | B<br>C    | B<br>C    | A+<br>A+<br>A | C<br>C     | A+<br>A<br>A |
| 20 | 60 hrs.                               |            |            |           |           |           |           |               |            | 20           |
|    | 90 hrs.                               |            |            |           |           |           |           |               |            |              |
|    | 120 hrs.                              |            |            |           |           |           |           |               |            |              |
|    | 150 hrs.                              |            |            |           |           |           |           |               |            |              |
|    | Number of rings stuck at—             |            |            |           |           |           |           |               |            |              |
|    | 60 hrs.                               | 1          | None       | None      | None      | None      | None      | None          | None       |              |
|    | 90 hrs.                               |            |            |           |           |           |           |               |            |              |
|    | 120 hrs.                              |            |            |           |           |           |           |               |            |              |
|    | 150 hrs.                              |            |            |           |           |           |           |               |            |              |
| 25 | Percent filling of oil ring slots at— |            |            |           |           |           |           |               |            | 25           |
|    | 60 hrs.                               | 90         | 5          | 5         | None      | 50        | 15        | None          | None       |              |
|    | 90 hrs.                               |            | 10         | 25        | 95        | 80        | 40        | None          | None       |              |
|    | 120 hrs.                              |            |            |           |           | 95        | 50        |               | None       |              |
|    | 150 hrs.                              |            |            |           |           |           | 60        |               | None       |              |
|    | Loss in weight of bearings, mgs. at—  |            |            |           |           |           |           |               |            |              |
| 30 | 60 hrs.                               | 22         | 1,075      | 1,176     | 1,062     | 306       | 288       | 70            | 86         |              |
|    | 90 hrs.                               |            | 1,385      | 1,460     | 1,248     | 367       | 402       | 107           | 138        | 30           |
|    | 120 hrs.                              |            |            |           |           | 432       | 520       |               |            |              |
|    | 150 hrs.                              |            |            |           |           |           | 630       |               | 259        |              |

In the foregoing table the symbols CaCPS, MgCPS, NiCPS and CoCPS denote respectively 35 calcium chlorphenyl stearate, magnesium chlorphenyl stearate, nickel chlorphenyl stearate and cobalt chlorphenyl stearate.

In view of the particular uses for which my 40 compounded lubricants are intended, it is apparent that of the salts included in the foregoing enumeration of the addition agents which may be employed, those which are readily oil soluble are the ones preferred for use. When these compounded oils are designed for use under 45 conditions where high temperatures are usually encountered, the addition agents should be stable at elevated temperatures. For use in crankcase lubricants for internal combustion engines, they should preferably be stable to the extent where there will be substantially no decomposition, when the lubricating composition is exposed to temperatures up to 250° F.

The addition agents which are to be selected 55 from the class described should be such that they are relatively non-corrosive with respect to the metallic surfaces with which they come in contact during use. Certain of the named addition agents may be found to be detrimentally 60 corrosive to certain sensitive bearing metals, in which case an appropriate corrosion inhibitor may be employed in conjunction therewith in the composition.

A lubricating composition prepared in accordance 65 with my invention and which is predominantly hydrocarbon oil may contain from an effective amount to 20% of the salt addition agent above identified. In general, it will be found that an amount as low as 1% will often be quite effective and that amounts in excess of 10% are seldom necessary. A preferred range of concentrations for the salt in the oil is from .25% to about 2%.

It is also within the contemplation of this 75 invention to provide the addition agents in the form of a concentrate in a suitable oil, said oil

for further blending with a lubricating oil in the proportions desired for the particular conditions of use.

While mineral oil, generally, is the principal 40 ingredient of the lubricant, it is not essential that it be the only ingredient other than the addition agent, provided that there be no additional ingredient which is incompatible with such addition agent. It is within the contemplation of this invention to include, if necessary or desirable, such other addition agents as are commonly added to improve the viscosity index or cold test of the lubricants; and a lubricating 45 composition according to this invention which also has a separate film-strength or oiliness increasing agent has been found to be especially effective.

When used in conjunction with a hydrocarbon 50 lubricating oil, it is obvious that, generally, only such amounts of the addition agent may be included as are soluble in the specified amount of oil. By the term "soluble," as herein used, it is intended to indicate the ability to form not 55 only true solutions but also any form of substantially permanently homogeneous composition when incorporated in mineral oil. With most of the compounds there is usually little difficulty, especially if the incorporation is effected in the 60 manner described in Cornell Patent No. 2,042,880, and since quite small percentages often give remarkably improved results, it is seldom of extreme 65 importance that the addition agents be oil-soluble in all proportions. Also, certain compounds are of value as gelling or bodying agents when used in amounts greater than are strictly soluble.

The addition agents above enumerated for use 70 in my compounded lubricants include certain ones which may be found to at least partially decompose under conditions of extreme stress such as the very high temperature encountered in certain classes of use, while others are quite stable even under such extreme conditions.

The use for which the lubricant is designed therefore determines the particular type of addition agent to be selected. A certain amount of decomposition, which proceeds at a relatively slow rate, is usually not harmful. Care should be exercised, however, to select for a particular set of operating conditions, an addition agent which in the oil base used, will not decompose under such operating conditions except at a low rate.

By the term "stable" as used herein in describing the addition agents is meant the characteristic of the addition agents which enables them to resist decomposition in the oil under the condition of use for which the lubricating composition is designed.

The lubricating compositions of this invention may be prepared by first preparing the salt and then dissolving the salt in the oil base, or they may be prepared by reacting the acid in solution in all or a portion of the oil with a suitable basic compound in order to form the desired salt directly in solution in oil. In the latter case, it is frequently desirable to remove the water formed by the reaction, or which may have been added with the basic compound, by some means such as by heating at atmospheric or sub-atmospheric pressure.

In case the salt to be used is water-insoluble, an alternative procedure is as follows:

An aqueous solution of a water-soluble salt of the acid is first prepared, for example by dissolving the acid in an aqueous solution of caustic soda or caustic potash. The aqueous salt solution is then emulsified with oil and a water-soluble salt containing the cation of the desired salt is added to the mixture. The desired salt is thus precipitated from the aqueous medium and subsequently or simultaneously dissolved by the oil medium. Separation of the aqueous and oil layers is then effected for example by settling or centrifuging preferably at elevated temperatures. Subsequent water-washing of the oil solution to remove traces of inorganic salts may be desirable, and removal of moisture may also be required.

This application is a continuation-in-part of my aforesaid co-pending applications Serial Numbers 737,070, 216,153 and 245,226.

Other modes of applying the principle of the invention may be employed, change being made as regards the details described, provided the features stated in any of the following claims or the equivalent of such be employed.

I therefore particularly point out and distinctly claim as my invention:

1. A lubricating composition containing as a principal lubricating constituent a major amount of a mineral lubricating oil with the properties of such composition affecting its use as a lubricant improved by incorporating therein a minor amount of a stable oil soluble salt of an aromatic acid of the type which may be produced by condensing chlorbenzene with oleic acid. 15

2. A lubricating composition containing as a principal lubricating constituent a major amount of a mineral lubricating oil with the properties of such composition affecting its use as a lubricant improved by incorporating therein a minor amount of a stable oil soluble metallic salt of an aromatic acid of the type which may be produced by condensing chlorbenzene with oleic acid. 20

3. A lubricating composition containing as a principal lubricating constituent a major amount of a mineral lubricating oil with the properties of such composition affecting its use as a lubricant improved by incorporating therein a minor amount of a stable oil soluble divalent metal salt 30 of an aromatic acid of the type which may be produced by condensing chlorbenzene with oleic acid. 25

4. A lubricating composition containing as a principal lubricating constituent a major amount of a mineral lubricating oil with the properties of such composition affecting its use as a lubricant improved by incorporating therein a minor amount of cobalt chlorphenyl stearate. 35

5. A lubricating composition containing as a principal lubricating constituent a major amount of a mineral lubricating oil with the properties of such composition affecting its use as a lubricant improved by incorporating therein a minor amount of nickel chlorphenyl stearate. 40 45

CARL F. PRUTTON.